



US008420705B2

(12) **United States Patent**  
**Greer, Jr.**

(10) **Patent No.:** **US 8,420,705 B2**  
(45) **Date of Patent:** **\*Apr. 16, 2013**

(54) **PARTICULATE MATERIALS FOR ACOUSTIC  
TEXTURE MATERIAL**

(75) Inventor: **Lester R. Greer, Jr.**, Sandpoint, ID (US)

(73) Assignee: **Homax Products, Inc.**, Bellingham, WA (US)

(\*) Notice: Subject to any disclaimer, the term of this patent is extended or adjusted under 35 U.S.C. 154(b) by 0 days.

This patent is subject to a terminal disclaimer.

(21) Appl. No.: **13/114,954**

(22) Filed: **May 24, 2011**

(65) **Prior Publication Data**

US 2011/0281030 A1 Nov. 17, 2011

**Related U.S. Application Data**

(63) Continuation of application No. 11/982,134, filed on Oct. 31, 2007, now Pat. No. 7,947,753, which is a continuation of application No. 11/027,219, filed on Dec. 29, 2004, now Pat. No. 7,374, 068.

(60) Provisional application No. 60/617,236, filed on Oct. 8, 2004.

(51) **Int. Cl.**  
**C08J 9/00** (2006.01)

(52) **U.S. Cl.**  
USPC ..... **521/78; 521/50**

(58) **Field of Classification Search** ..... 521/50,  
521/78

See application file for complete search history.

(56) **References Cited**

**U.S. PATENT DOCUMENTS**

2,353,318 A 7/1944 Scheller  
2,565,954 A 8/1951 Dey

(Continued)

**FOREIGN PATENT DOCUMENTS**

|    |         |        |
|----|---------|--------|
| CA | 1210371 | 8/1986 |
| CA | 2145129 | 9/1995 |

(Continued)

**OTHER PUBLICATIONS**

Homax Products, Inc., "Homax Easy Touch Spray Texture Brochure", Mar. 1992, 1 page.

(Continued)

*Primary Examiner* — Mark Eashoo

*Assistant Examiner* — Melissa Rioja

(74) *Attorney, Agent, or Firm* — Michael R. Schacht; Schacht Law Office, Inc.

(57) **ABSTRACT**

A composition for forming a textured coating on drywall material, where the textured coating substantially matches a pre-existing acoustic texture material on the drywall material, comprises acoustic texture material and propellant material. The acoustic texture material comprises a base portion the base portion is capable of existing in a flowable state and a hardened state, and a particulate portion the particulate portion comprises discrete, visible particles of solidified urethane foam having irregular shapes. The propellant material comprises a hydrocarbon propellant. The particles of urethane foam are distributed throughout the acoustic texture material when the base portion is in the flowable state. The irregular shapes of the particulate portion are substantially the same when the base portion is in the flowable state and in the hardened state. The base portion is capable of securing the discrete, visible, particles of solidified urethane foam to the drywall material when the base portion is in the hardened state.

**5 Claims, 3 Drawing Sheets**



# US 8,420,705 B2

Page 2

| U.S. PATENT DOCUMENTS |         |                   |                                    |
|-----------------------|---------|-------------------|------------------------------------|
| 2,686,652 A           | 8/1954  | Carlson et al.    | 5,188,295 A                        |
| 2,723,200 A           | 11/1955 | Pyenson           | 5,211,317 A                        |
| 2,763,406 A           | 9/1956  | Countryman        | 5,310,095 A                        |
| 2,764,454 A           | 9/1956  | Edelstein         | 5,312,888 A                        |
| 2,785,926 A           | 3/1957  | Lataste           | 5,341,970 A                        |
| 2,831,618 A           | 4/1958  | Soffer et al.     | 5,409,148 A                        |
| 2,839,225 A           | 6/1958  | Soffer et al.     | D358,989 S                         |
| 2,932,434 A           | 4/1960  | Abplanalp         | 5,421,519 A                        |
| 2,965,270 A           | 12/1960 | Soifer et al.     | 5,450,983 A                        |
| 3,191,809 A           | 6/1965  | Schultz et al.    | 5,476,879 A                        |
| 3,196,819 A           | 7/1965  | Lechner et al.    | 5,489,048 A                        |
| 3,198,394 A           | 8/1965  | Lefer             | 5,505,344 A                        |
| 3,346,195 A           | 10/1967 | Groth             | 5,524,798 A                        |
| 3,415,425 A           | 12/1968 | Knight et al.     | 5,639,026 A                        |
| 3,433,391 A           | 3/1969  | Krizka et al.     | 5,645,198 A                        |
| 3,450,314 A           | 6/1969  | Gross             | 5,655,691 A                        |
| 3,467,283 A           | 9/1969  | Kinnavy           | 5,695,788 A                        |
| 3,482,738 A           | 12/1969 | Bartels           | 5,715,975 A                        |
| 3,544,258 A           | 12/1970 | Presant et al.    | 5,727,736 A                        |
| 3,548,564 A           | 12/1970 | Bruce et al.      | 5,921,446 A                        |
| 3,592,359 A           | 7/1971  | Marraffino        | 5,934,518 A                        |
| 3,700,136 A           | 10/1972 | Ruekberg          | 5,941,462 A                        |
| 3,776,702 A           | 12/1973 | Chant             | 6,000,583 A                        |
| 3,788,521 A           | 1/1974  | Laaewe            | 6,095,435 A                        |
| 3,806,005 A           | 4/1974  | Prussin et al.    | 6,112,945 A                        |
| 3,813,011 A           | 5/1974  | Harrison et al.   | 6,116,473 A                        |
| 3,828,977 A           | 8/1974  | Borchert          | 6,152,335 A                        |
| 3,862,705 A           | 1/1975  | Beres et al.      | 6,168,093 B1                       |
| 3,913,842 A           | 10/1975 | Singer            | D438,111 S                         |
| 3,932,973 A           | 1/1976  | Moore             | 6,225,393 B1                       |
| 3,938,708 A           | 2/1976  | Burger            | 6,276,570 B1                       |
| 3,989,165 A           | 11/1976 | Shaw et al.       | 6,299,679 B1                       |
| 3,992,003 A           | 11/1976 | Visceglia et al.  | 6,328,185 B1                       |
| 4,010,134 A *         | 3/1977  | Braunisch et al.  | 6,352,184 B1                       |
| 4,032,064 A           | 6/1977  | Giggard           | 252/62                             |
| 4,045,860 A           | 9/1977  | Winckler          | 6,362,302 B1                       |
| 4,089,443 A           | 5/1978  | Zrinyi            | 6,375,036 B1                       |
| 4,117,951 A           | 10/1978 | Winckler          | 6,382,474 B1                       |
| 4,148,416 A           | 4/1979  | Gunn-Smith        | 6,386,402 B1                       |
| 4,154,378 A           | 5/1979  | Paoletti et al.   | 6,395,794 B2                       |
| RE30,093 E            | 9/1979  | Burger            | 6,399,687 B2                       |
| 4,171,757 A           | 10/1979 | Diamond           | 6,415,964 B2                       |
| 4,185,758 A           | 1/1980  | Giggard           | 6,446,842 B2                       |
| 4,187,959 A           | 2/1980  | Pelton            | 6,447,561 B2                       |
| 4,198,365 A           | 4/1980  | Pelton            | 6,536,633 B2                       |
| 4,238,264 A           | 12/1980 | Pelton            | 6,641,005 B1                       |
| 4,275,172 A           | 6/1981  | Barth et al.      | 6,641,864 B2                       |
| 4,293,353 A           | 10/1981 | Pelton et al.     | 6,659,312 B1                       |
| 4,308,973 A           | 1/1982  | Irland            | 6,666,352 B1                       |
| 4,322,020 A           | 3/1982  | Stone             | 6,712,238 B1                       |
| 4,346,743 A           | 8/1982  | Miller            | 6,726,066 B2                       |
| 4,370,930 A           | 2/1983  | Strasser et al.   | 6,797,051 B2                       |
| 4,401,271 A           | 8/1983  | Hansen            | 6,883,688 B1                       |
| 4,401,272 A           | 8/1983  | Merton et al.     | 6,905,050 B1                       |
| 4,411,387 A           | 10/1983 | Stern et al.      | 6,910,608 B2                       |
| 4,417,674 A           | 11/1983 | Giuffredi         | 6,913,407 B2                       |
| 4,438,221 A           | 3/1984  | Fracalossi et al. | 7,014,073 B1                       |
| 4,442,959 A           | 4/1984  | Del Bon et al.    | 7,059,497 B2                       |
| 4,641,765 A           | 2/1987  | Diamond           | 7,163,962 B2                       |
| 4,683,246 A           | 7/1987  | Davis et al.      | 7,189,022 B1                       |
| 4,793,162 A           | 12/1988 | Emmons            | 7,192,985 B2                       |
| 4,839,393 A           | 6/1989  | Buchanan et al.   | 7,226,001 B1                       |
| 4,854,482 A           | 8/1989  | Bergner           | 7,226,232 B2                       |
| 4,870,805 A           | 10/1989 | Morane            | 7,232,047 B2                       |
| 4,896,832 A           | 1/1990  | Howlett           | 7,240,857 B1                       |
| 4,940,171 A           | 7/1990  | Gilroy            | 7,278,590 B1                       |
| 4,949,871 A           | 8/1990  | Flanner           | 7,337,985 B1                       |
| 4,955,545 A           | 9/1990  | Stern et al.      | 7,374,068 B2 *                     |
| 4,961,537 A           | 10/1990 | Stern             | 7,481,338 B1                       |
| 4,969,577 A           | 11/1990 | Werdeing          | 7,487,893 B1 *                     |
| 5,007,556 A           | 4/1991  | Lover             | 7,500,621 B2                       |
| 5,037,011 A           | 8/1991  | Woods             | 7,597,274 B1                       |
| 5,038,964 A           | 8/1991  | Bouix             | 7,600,659 B1                       |
| 5,059,187 A           | 10/1991 | Sperry et al.     | 7,624,932 B1                       |
| 5,069,390 A           | 12/1991 | Stern et al.      | 7,673,816 B1                       |
| 5,115,944 A           | 5/1992  | Nikolich          | 7,677,420 B1 *                     |
| 5,126,086 A           | 6/1992  | Stoffel           | 7,744,299 B1                       |
| 5,188,263 A           | 2/1993  | Woods             | 7,784,649 B2 *                     |
|                       |         |                   | 2/1993 Stern et al.                |
|                       |         |                   | 5/1993 Diamond et al.              |
|                       |         |                   | 5/1994 Stern et al.                |
|                       |         |                   | 5/1994 Nafziger et al.             |
|                       |         |                   | 8/1994 Woods                       |
|                       |         |                   | 4/1995 Stern et al.                |
|                       |         |                   | 6/1995 Woods                       |
|                       |         |                   | 6/1995 Woods                       |
|                       |         |                   | 9/1995 Stern et al.                |
|                       |         |                   | 12/1995 Woods et al.               |
|                       |         |                   | 2/1996 Stern et al.                |
|                       |         |                   | 4/1996 Woods                       |
|                       |         |                   | 12/1997 Stern et al.               |
|                       |         |                   | 2/1998 Stern et al.                |
|                       |         |                   | 3/1998 Tryon                       |
|                       |         |                   | 7/1999 Stern                       |
|                       |         |                   | 8/1999 Stern et al.                |
|                       |         |                   | 8/1999 Sandor                      |
|                       |         |                   | 12/1999 Stern et al.               |
|                       |         |                   | 8/2000 Greer, Jr. et al.           |
|                       |         |                   | 9/2000 Woods                       |
|                       |         |                   | 11/2000 Stern et al.               |
|                       |         |                   | 1/2001 Greer, Jr. et al.           |
|                       |         |                   | 2/2001 Woods                       |
|                       |         |                   | 5/2001 Woods                       |
|                       |         |                   | 3/2002 Stern et al.                |
|                       |         |                   | 3/2002 Boddie                      |
|                       |         |                   | 4/2002 Woods                       |
|                       |         |                   | 5/2002 Woods et al.                |
|                       |         |                   | 5/2002 Woods                       |
|                       |         |                   | 5/2002 Lucas et al.                |
|                       |         |                   | 6/2002 Woods                       |
|                       |         |                   | 7/2002 Woods                       |
|                       |         |                   | 9/2002 Stern et al.                |
|                       |         |                   | 11/2002 Braun et al.               |
|                       |         |                   | 3/2003 Stern et al.                |
|                       |         |                   | 11/2003 Stern et al.               |
|                       |         |                   | 11/2003 Woods                      |
|                       |         |                   | 12/2003 Stern et al.               |
|                       |         |                   | 12/2003 Woods                      |
|                       |         |                   | 3/2004 Mills                       |
|                       |         |                   | 6/2004 Woods                       |
|                       |         |                   | 9/2004 Woods                       |
|                       |         |                   | 4/2005 Stern et al.                |
|                       |         |                   | 6/2005 Stern et al.                |
|                       |         |                   | 6/2005 Greer, Jr. et al.           |
|                       |         |                   | 7/2005 Greer et al.                |
|                       |         |                   | 3/2006 Stern et al.                |
|                       |         |                   | 6/2006 Woods                       |
|                       |         |                   | 1/2007 Woods                       |
|                       |         |                   | 3/2007 Greer, Jr. et al.           |
|                       |         |                   | 3/2007 Woods                       |
|                       |         |                   | 7/2007 Stern et al.                |
|                       |         |                   | 6/2007 Stern et al.                |
|                       |         |                   | 6/2007 Greer, Jr. et al.           |
|                       |         |                   | 3/2008 Greer, Jr. et al.           |
|                       |         |                   | 5/2008 Greer, Jr. .... 222/402.1   |
|                       |         |                   | 1/2009 Stern et al.                |
|                       |         |                   | 2/2009 Greer et al. .... 222/402.1 |
|                       |         |                   | 3/2009 Tryon et al.                |
|                       |         |                   | 10/2009 Stern et al.               |
|                       |         |                   | 10/2009 Greer, Jr. et al.          |
|                       |         |                   | 12/2009 Greer, Jr. et al.          |
|                       |         |                   | 3/2010 Stern et al.                |
|                       |         |                   | 3/2010 Greer et al. .... 222/402.1 |
|                       |         |                   | 6/2010 Greer, Jr. et al.           |
|                       |         |                   | 8/2010 Greer, Jr. .... 222/402.1   |

|              |      |         |                             |
|--------------|------|---------|-----------------------------|
| 7,845,523    | B1   | 12/2010 | Greer, Jr. et al.           |
| 7,947,753    | B2 * | 5/2011  | Greer, Jr. .... 521/78      |
| 8,028,864    | B2   | 10/2011 | Stern et al.                |
| 8,033,484    | B2   | 10/2011 | Tryon et al.                |
| 8,038,077    | B1   | 10/2011 | Greer, Jr. et al.           |
| 8,042,713    | B2 * | 10/2011 | Greer et al. .... 222/402.1 |
| 8,157,135    | B2   | 4/2012  | Stern et al.                |
| 2001/0002676 | A1   | 6/2001  | Woods                       |
| 2002/0119256 | A1   | 8/2002  | Woods                       |
| 2004/0099697 | A1 * | 5/2004  | Woods .... 222/402.1        |
| 2004/0195277 | A1   | 10/2004 | Woods                       |
| 2005/0161531 | A1   | 7/2005  | Greer, Jr. et al.           |
| 2005/0236436 | A1   | 10/2005 | Woods                       |
| 2006/0079588 | A1 * | 4/2006  | Greer, Jr. .... 521/78      |
| 2006/0180616 | A1   | 8/2006  | Woods                       |
| 2006/0219808 | A1   | 10/2006 | Woods                       |
| 2006/0219811 | A1   | 10/2006 | Woods                       |
| 2006/0273207 | A1   | 12/2006 | Woods                       |
| 2007/0119984 | A1   | 5/2007  | Woods                       |
| 2007/0219310 | A1   | 9/2007  | Woods                       |
| 2007/0235563 | A1   | 10/2007 | Woods                       |
| 2007/0260011 | A1   | 11/2007 | Woods                       |
| 2011/0281030 | A1   | 11/2011 | Greer, Jr.                  |
| 2012/0064249 | A1   | 3/2012  | Greer, Jr.                  |
| 2012/0080446 | A1   | 4/2012  | Tryon et al.                |

## FOREIGN PATENT DOCUMENTS

|    |         |         |
|----|---------|---------|
| CA | 2090185 | 10/1998 |
| CA | 2224042 | 6/1999  |
| CA | 2291599 | 6/2000  |
| CA | 2381994 | 2/2001  |
| CA | 2065534 | 8/2003  |
| CA | 2448794 | 5/2004  |
| CA | 2504509 | 10/2005 |
| CA | 2504513 | 10/2005 |
| DE | 3806991 | 9/1989  |
| GB | 2418959 | 4/2006  |

## OTHER PUBLICATIONS

USPTO, Office Action U.S. Appl. No. 11/982,133, Jan. 28, 2009, 6 pages.  
 Schacht Law Office, Inc., Response to Jan. 28, 2009 Office Action, Feb. 27, 2009, 2 pages.  
 USPTO, Office Action U.S. Appl. No. 11/982,133, Mar. 27, 2009, 12 pages.  
 Schacht Law Office, Inc., Response to Mar. 27, 2009 Office Action, Jul. 27, 2009, 9 pages.  
 USPTO, Office Action U.S. Appl. No. 11/982,133, Nov. 30, 2009, 4 pages.  
 Schacht Law Office, Inc., Response to Nov. 30, 2009 Office Action, Mar. 1, 2010, 10 pages.  
 USPTO, Office Action U.S. Appl. No. 11/982,133, May 18, 2010, 7 pages.  
 USPTO, Office Action U.S. Appl. No. 12,859,195, Jan. 20, 2011, 6 pages.  
 Schacht Law Office, Inc., Response to Jan. 20, 2011 Office Action, Apr. 20, 2011, 10 pages.  
 USPTO, Notice of Allowance U.S. Appl. No. 12/859,195, Jul. 15, 2011, 20 pages.  
 USPTO, Office Action U.S. Appl. No. 13/280,924, Mar. 26, 2012, 6 pages.  
 USPTO, Office Action U.S. Appl. No. 11/413,659, May 29, 2007, 12 pages.  
 Schacht Law Office, Inc., Response to May 29, 2007 Office Action, Aug. 29, 2007, 16 pages.  
 USPTO, Office Action U.S. Appl. No. 11/413,659, Nov. 15, 2007, 5 pages.  
 Schacht Law Office, Inc., Response to Nov. 15, 2007 Office Action, Feb. 15, 2008, 8 pages.  
 USPTO, Office Action U.S. Appl. No. 11/413,659, Mar. 17, 2008, 7 pages.  
 Schacht Law Office, Inc., Response to Mar. 17, 2008 Office Action, Jun. 17, 2008, 9 pages.  
 USPTO, Notice of Allowance U.S. Appl. No. 11/413,659, Sep. 30, 2008, 8 pages.

\* cited by examiner

FIG. 1



FIG. 2



FIG. 3



FIG. 4



FIG. 5



FIG. 6



## 1

PARTICULATE MATERIALS FOR ACOUSTIC  
TEXTURE MATERIAL

## RELATED APPLICATIONS

This application, U.S. patent application Ser. No. 13/114,954 filed May 24, 2011, is a continuation of U.S. patent application Ser. No. 11/982,134 filed Oct. 31, 2007, now U.S. Pat. No. 7,947,753 which issued May 24, 2011.

U.S. patent application Ser. No. 11/982,134 is a continuation of U.S. patent application Ser. No. 11/027,219 filed Dec. 29, 2004, now U.S. Pat. No. 7,374,068 which issued May 20, 2008.

U.S. patent application Ser. No. 11/027,219 claims benefit of U.S. Provisional Patent Application Ser. No. 60/617,236 filed Oct. 8, 2004.

All related applications cited in this Related Applications section, including the subject matter thereof, are incorporated herein by reference.

## TECHNICAL FIELD

The present invention relates to particulate materials for use in acoustic texture material and, more particularly, to particulate materials that may be used in acoustic texture material formulated to be dispensed from aerosol dispensers.

## BACKGROUND

Interior walls are formed by sheets of drywall material that are secured to the framing of a building. The seams between adjacent sheets of drywall material are taped, mudded, and sanded to obtain a substantially flat, smooth drywall surface. The drywall surface is coated with primer and paint to obtain a finished surface.

In some situations, a separate texture layer is applied to the drywall surface prior to painting. The texture layer is formed by spraying texture material onto the drywall surface. Texture material is a coating material that, when sprayed, does not form a smooth, thin coating. Instead, texture material is applied in discrete drops or globs that dry to form a bumpy, irregular textured surface.

Texture materials can be applied using any one of a number of application systems. During new construction, texture materials are commonly applied in a stream of compressed air using commercial hopper gun systems. For touch up or repair, texture material is commonly applied using hand operated pneumatic pumps or aerosol dispensing systems. Varying the parameters of the application system varies the size and spacing of the bumps to vary the look of the textured surface.

One specific form of texture material is commonly referred to as "acoustic" or "popcorn" texture material. In addition to a coating material, acoustic texture material further comprises an aggregate material. When the acoustic texture material is applied using commercial hopper guns, the aggregate material is conventionally formed by polystyrene chips. However, as will be described in detail below, chips made of polystyrene foam are dissolved by hydrocarbon aerosol propellant materials.

Accordingly, aerosol dispensing systems for dispensing small amounts of acoustic texture material for repair or touch-up purposes use one of two approaches. The first approach is to mix a liquid hydrocarbon aerosol propellant material with chips made from materials other than polystyrene. However, when chips made of materials other than polystyrene foam are used, the appearance and function of the texture surface may be different from that of the surrounding surface.

## 2

The second approach is to combine polystyrene chips with a propellant material formed by a pressurized inert gas such as nitrogen or air. This second approach allows the use of a conventional acoustic texture material including polystyrene chips. However, the use of a pressurized inert gas causes the acoustic texture material to be dispensed very quickly. The use of pressurized inert gas as a propellant can make it difficult for a non-professional to control the application of the acoustic texture material.

The need thus exists for improved systems and methods for dispensing small quantities of acoustic texture material for the purpose of touch-up or repair.

## SUMMARY

The present invention may be embodied as a composition for forming a textured coating on drywall material, where the textured coating substantially matches a pre-existing acoustic texture material on the drywall material, comprising acoustic texture material and propellant material. The acoustic texture material comprises a base portion the base portion is capable of existing in a flowable state and a hardened state, and a particulate portion the particulate portion comprises discrete, visible particles of solidified urethane foam having irregular shapes. The propellant material comprises a hydrocarbon propellant. The particles of urethane foam are distributed throughout the acoustic texture material when the base portion is in the flowable state. The irregular shapes of the particulate portion are substantially the same when the base portion is in the flowable state and in the hardened state. The base portion is capable of securing the discrete, visible, particles of solidified urethane foam to the drywall material when the base portion is in the hardened state.

The present invention may also be embodied as a method of forming a textured coating on drywall material such that the textured coating substantially matches a pre-existing acoustic texture material on the drywall material comprising the following steps. Acoustic texture material comprising a base portion capable of existing in a flowable state and a hardened state and a particulate portion comprising discrete, visible particles of solidified urethane foam having irregular shapes is provided. The acoustic texture material is arranged within an aerosol assembly such that the particles of urethane foam are distributed throughout the base portion when the base portion is in the flowable state. Propellant material comprising a hydrocarbon propellant is arranged within the aerosol assembly. The aerosol assembly is operated such that the propellant material forces the acoustic texture material out of the aerosol assembly and onto the drywall material and the base portion changes to the hardened state such that the discrete, visible, particles of solidified urethane are secured to the drywall material.

## BRIEF DESCRIPTION OF THE DRAWINGS

FIG. 1 is a section view of a first embodiment of an aerosol dispensing system containing acoustic texture material incorporating particulate material of the present invention;

FIG. 2 is a section view of a second embodiment of an aerosol dispensing system containing acoustic texture material incorporating particulate material of the present invention;

FIG. 3 is an elevation view depicting the use of one or both of the first and second aerosol dispensing systems of FIGS. 1 and 2 being used to deposit acoustic texture material to a surface;

FIG. 4 is a section view of the acoustic texture material after it has been deposited on the surface; and

FIGS. 5 and 6 are bottom plan views of the surface before and after the acoustic texture material has been deposited thereon.

#### DETAILED DESCRIPTION

Referring initially to FIG. 1 of the drawing, depicted at 20a therein is a first embodiment of an aerosol system for depositing on a surface 22 (FIGS. 3-6) acoustic texture material 24 incorporating particulate material 26 of the present invention. FIG. 5 illustrates a target portion 28 of the surface 22 on which acoustic texture material 24 is to be deposited.

The example aerosol system 20a comprises a container assembly 30, a valve assembly 32, a collection assembly 34, and an outlet assembly 36. The container 30 defines a product chamber 40 in which the acoustic texture material 24 comprising the particulate material 26 is contained. A first portion 42 of the chamber 40 is occupied by the acoustic texture material 24, while a second portion 44 of the chamber 40 is occupied by a pressurized propellant material 46. The example container assembly 30 comprises a can member 50 and a cup member 52.

The valve assembly 32 is mounted in a cup opening 34 define by the cup member 52 and operates in a closed configuration (shown) and an open configuration. In the open configuration, the valve assembly 32 defines a dispensing passageway that allows fluid communication between the interior and the exterior of the container assembly 30.

The outlet assembly 36 comprises an actuator member 60 that causes acoustic texture material 24 to be dispensed by the system 20 in a fan shaped spray as will be described in further detail below. The actuator member 60 is mounted on the valve assembly 32 such that displacing the outlet member 60 towards the valve assembly 32 places the valve assembly in the open configuration.

The example valve assembly 32 comprises a valve seat 70, a valve stem 72, a valve housing 74, a dip tube 76, and a valve spring 78. The valve seat 70 defines a seat opening 70a and is supported by the cup member 52. The valve stem 72 defines a valve stem opening 72a and a valve surface 72b. The valve stem 72 is supported by the valve seat 70 such that the valve stem moves within the valve stem opening 72a between first and second positions, with the first position being shown in FIG. 1.

The valve housing 74 is supported by the valve seat 70 within the product chamber 40. The valve housing 74 further supports the dip tube 76 such that the acoustic texture material 24 within can flow into the valve housing 74 when the can is upright. The valve spring 78 is supported by the valve housing 74 such that the spring 78 biases the valve stem 72 into the first position. The valve stem 72 supports the outlet assembly 36 such that depressing the actuator member 60 towards the cup member 52 forces the valve stem 72 into the second position (not shown) against the force of the valve spring 78.

The valve assembly 32 thus operates in the closed configuration and the open configuration as follows. When no force is applied to the actuator member 60, the valve spring 78 forces the valve surface 72b against the valve seat 70 to prevent fluid from flowing through the valve stem opening 72a. When a force is applied to the actuator member 60, the valve surface 72b is forced away from the valve seat 70 such that fluid can flow from the interior of the valve housing 74 through the valve stem opening 72a and thus out of the product chamber 40.

Referring now to FIG. 2 of the drawing, depicted at 20b therein is a first embodiment of an aerosol system that may also be used to deposit the acoustic texture material 24 incorporating particulate material 26 of the present invention on the target portion 28 of the surface 22.

The example aerosol system 20b comprises a container assembly 130, a valve assembly 132, a collection assembly 134, and an outlet assembly 136. The container 130 defines a product chamber 140 in which the acoustic texture material 24 comprising the particulate material 26 is contained. A first portion 142 of the chamber 140 is occupied by the acoustic texture material 24, while a second portion 144 of the chamber 140 is occupied by a pressurized propellant material 146. The example container assembly 130 comprises a can member 150 and a cup member 152.

The valve assembly 132 is mounted in a cup opening 134 define by the cup member 152 and operates in a closed configuration (shown) and an open configuration. In the open configuration, the valve assembly 132 defines a dispensing passageway that allows fluid communication between the interior and the exterior of the container assembly 130.

The outlet assembly 136 comprises an actuator member 160 that causes acoustic texture material 24 to be dispensed by the system 20 in a fan shaped spray as will be described in further detail below. The actuator member 160 is mounted on the valve assembly 132 such that displacing the outlet member 160 towards the valve assembly 132 places the valve assembly in the open configuration.

The example valve assembly 132 comprises a valve seat 170, a valve stem 172, a valve housing 174, a dip tube 176, and a valve spring 178. The valve seat 170 defines a seat opening 170a and is supported by the cup member 152. The valve stem 172 defines a valve stem opening 172a and a valve surface 172b. The valve stem 172 is supported by the valve seat 170 such that the valve stem moves within the valve stem opening 172a between first and second positions, with the first position being shown in FIG. 1.

The valve housing 174 is supported by the valve seat 170 within the product chamber 140. The valve housing 174 further supports the dip tube 176 such that the acoustic texture material 124 within can flow into the valve housing 174 when the can is upright. The valve spring 178 is supported by the valve housing 174 such that the spring 178 biases the valve stem 172 into the first position. The valve stem 172 supports the outlet assembly 136 such that depressing the actuator member 160 towards the cup member 152 forces the valve stem 172 into the second position (not shown) against the force of the valve spring 178.

The valve assembly 132 thus operates in the closed configuration and the open configuration as follows. When no force is applied to the actuator member 160, the valve spring 178 forces the valve surface 172b against the valve seat 170 to prevent fluid from flowing through the valve stem opening 172a. When a force is applied to the actuator member 160, the valve surface 172b is forced away from the valve seat 170 such that fluid can flow from the interior of the valve housing 174 through the valve stem opening 172a and thus out of the product chamber 140.

Turning now to FIGS. 3-6, the use of the aerosol dispensing systems 20a and 20b will now be described in further detail. These dispensing systems 20a and 20b are used in the same manner and are both identified by reference character 20 in FIGS. 3-6.

As shown in FIG. 3, the dispensing system 20 deposits a fan-shaped spray of acoustic texture material 24 on the target portion 28 of the wall 22. As shown in FIGS. 4 and 6, the acoustic texture material 24 covers the target portion 28 to

match the pre-existing acoustic texture material on the surface 22 surrounding the target portion 28.

Referring for a moment back to FIGS. 1 and 2, it can be seen that, in addition to the particulate material 26, the acoustic texture material comprises a base portion 220 in the form of a flowable liquid. The base portion 220 of the particulate material conventionally comprises a carrier, a filler, and a binder.

In some aerosol systems, the propellant material 46,146 is simply an inert pressurized gas such as air or nitrogen. In other aerosol systems, the propellant material 46,146 is a material, referred to herein as bi-phase propellant material, that exists in both gaseous and liquid phases within the container assembly 30,130. The liquid phase of the propellant material 46,146 forms a part of the base portion 220, while the gaseous phase propellant material 46,146 occupies the pressurized portion 44 of the container assembly 30,130.

As the acoustic texture material 24 is dispensed, the pressure within the pressurized portion 44,144 of the container assemblies 30,130 drops. Under these conditions, a portion of the bi-phase propellant material 46,146 in the liquid phase gasifies to re-pressurize the pressurized portion 44,144 of the container assembly 30,130. The pressure within the pressurized portion 44,144 is thus under most conditions sufficient to force the acoustic texture material 24 out of the container assembly 30,130 along the dispensing passageway when the valve assembly 32,132 is in the open configuration. The propellant material 46,146 may thus be a pressurized inert gas such as air or nitrogen.

However, the present invention is of particular significance when the propellant material is a bi-phase propellant material such as di-methyl ethylene (DME) or any one of a number of hydrocarbon propellants such as those available in the industry as A-40 and A-70. The advantage of using bi-phase propellant materials is that the pressure within the pressurized portion 44,144 of the container assembly 30,130 is kept at a relatively constant, relatively low level as the level of acoustic texture material 24 drops. This constant, low level pressure allows the texture material 24 to be dispensed in many small bursts instead of in a few large bursts, as is the case when pressurized inert gases are used as the propellant material 46,146.

Many particulate materials 26 suitable for use in acoustic texture materials are incompatible with bi-phase propellant materials. For example, as described above polystyrene chips are commonly used in acoustic texture materials dispensed using commercial hopper guns. However, polystyrene chips dissolve in the bi-phase propellant materials of which the Applicant is aware.

The Applicant has discovered that urethane foam materials and melamine foam materials may be used as the particulate material 26 with bi-phase propellant materials such as DME and hydrocarbon propellants such as A-40 and A-70. Melamine foam materials in particular are easily chopped up using conventional material processors (e.g., a food blender) into irregular shapes that match the appearance and function of polystyrene chips. Melamine foam materials are already commonly used in building applications and have desirable fire retardant, thermal, and acoustic properties.

To manufacture the acoustic texture material 24, the base portion 220 may be the same as a conventional base used in commercially available acoustic texture materials. Instead of polystyrene chips, however, urethane and/or melamine foam is chopped up into particles of an appropriate size and use as

the particulate. In addition, a bi-phase propellant material is used to form part of the carrier portion of the base portion 220.

The Applicant has thus determined that a conventional base portion using melamine foam chips and DME as a propellant is commercially practical and obtains acceptable aesthetic and functional results. Appropriate adjustments in the liquids used as the carrier in a conventional acoustic texture material formulation may be required to obtain a desired consistency of the acoustic texture material 24 as it is deposited on the surface 22.

What is claimed is:

1. A composition for forming a textured coating on drywall material, where the textured coating substantially matches a pre-existing acoustic texture material on the drywall material, comprising:

acoustic texture material comprising

a base portion the base portion is capable of existing in a flowable state and a hardened state, and

a particulate portion the particulate portion comprises discrete, visible particles of solidified urethane foam having irregular shapes

propellant material comprising a hydrocarbon propellant; wherein

the particles of urethane foam are distributed throughout the acoustic texture material when the base portion is in the flowable state;

the irregular shapes of the particulate portion are substantially the same when the base portion is in the flowable state and in the hardened state; and the base portion is capable of securing the discrete, visible, particles of solidified urethane foam to the drywall material when the base portion is in the hardened state.

2. A composition as recited in claim 1, in which the hydrocarbon propellant is DME.

3. A method of forming a textured coating on drywall material such that the textured coating substantially matches a pre-existing acoustic texture material on the drywall material, comprising the steps of:

providing acoustic texture material comprising

a base portion capable of existing in a flowable state and a hardened state, and

a particulate portion comprising discrete, visible particles of solidified urethane foam having irregular shapes;

arranging within an aerosol assembly the acoustic texture material such that the particles of urethane foam are distributed throughout the base portion when the base portion is in the flowable state;

arranging within the aerosol assembly propellant material comprising a hydrocarbon propellant; and

operating the aerosol assembly such that

the propellant material forces the acoustic texture material out of the aerosol assembly and onto the drywall material, and

the base portion changes to the hardened state such that the discrete, visible, particles of solidified urethane are secured to the drywall material.

4. A method as recited in claim 3, in which the hydrocarbon propellant is DME.

5. A method as recited in claim 3, in which the irregular shapes of the urethane foam particles are substantially the same when the base portion of the acoustic texture material is in the flowable state and in the hardened state.